

1

3,071,856

RAZOR BLADE AND METHOD OF MAKING SAME  
Irwin W. Fischbein, 18 Joyce Road, Hyde Park, Mass.  
No Drawing. Filed Dec. 31, 1959, Ser. No. 863,109  
15 Claims. (Cl. 30—346)

This invention relates to safety razor blades, either single edged or double edged, and pertains more specifically to an improved safety razor blade with a cutting edge on which is an adherent coating comprising a fluorocarbon which improves the shaving effectiveness of the blade edge and to the method of making such blades.

Conventional steel safety razor blades to which the present invention may be applied to produce improved blades are from 0.003 to 0.015 inch thick and have wedge-shaped cutting edges, the included solid angle of which is greater than 14° and less than 35°. The faces or sides of some such cutting edges extend back from the edge for a distance up to as much as 0.1 inch or even more. Each face need not be a single planar uninterrupted continuous surface or "facet," but may consist of two or more "facets" formed by successive grinding or honing operations and intersecting each other along zones generally parallel to the ultimate edge. The final facet, i.e., the facet immediately adjacent the ultimate edge, may have a width as little as 0.0003 inch or even less as compared to the diameter of a beard hair which averages about 0.004 to 0.005 inch, while the thickness of the ultimate edge itself is generally less than 6000 Angstrom units and preferably less than 2500 Angstrom units. The steel of which the blade edge is composed may be either carbon steel or hardenable stainless steel. In either case it is hardened by a suitable heat-treating process. There is a limit to the extent to which the blade subsequently may be heated since excessive reheating will lead to loss of hardness. As a general rule the hardened metal blade edges cannot be subjected to a temperature above about 400° F. for more than five minutes without risk that some objectionable tempering or softening of the steel will occur. However, the coating may also be applied to blades having cutting edges of (or coated with) metals or metal alloys other than steel or stainless steel.

Conventional razor blades despite their sharpness cannot be employed for shaving a dry beard without excessive discomfort and pain, and it is as a practical matter necessary to employ with them a beard-softening agent such as water and/or a shaving cream or soap. The pain and irritation produced by shaving dry are due to the excessive force required to draw the cutting edge of the blade through the unsoftened beard hairs, which force is transmitted to the nerves in the skin adjacent the hair follicles from which the beard hairs extend, and, as is well known, the irritation produced by excessive pulling of these hairs may continue for a considerable period of time after the pulling has ceased. Although a variety of materials have been applied both to the cutting edges of blades and to the beard hair in an effort to reduce the pull, the only materials which have been found commercially useful prior to the present invention are those which soften the beard hair itself.

Applicant has discovered that by providing on the cutting edge of a safety razor blade a thin integument of a fluorocarbon which is adherent to the substrate, the blade exhibits a remarkable increase in shaving effectiveness. This improvement is characterized by a decrease in pull; that is, a decrease in the force required to cut the beard hairs, which manifests itself in markedly increased ease and smoothness of shaving, making it possible, if desired, to abbreviate the customary beard-softening step which precedes shaving, since softening of the beard is not so important as in the case of conventional blades. The

2

blades of the present invention when tested under carefully controlled conditions off the face require much less force to cut water-softened hair than do similar blades without the integument. This reduction in pull may persist during several successive shaves with the same blade cutting edge, although it does not persist indefinitely.

The fluorocarbon integument or coating may extend over the entire wedge faces back from the ultimate edge or even farther, or it may cover only the portion of the final facet immediately adjacent to the ultimate edge. The precise thickness of the integument does not appear to be critical, a thin continuous adherent coating having a thickness of the order of an oriented monolayer of molecules having been found effective for the purpose of the present invention. The thickness of the integument need not be uniform throughout its extent.

The fluorocarbon materials which may be used in practicing the present invention are solid materials and include a variety of solid polymers of tetrafluoroethylene containing a chain of carbon atoms including a plurality of (—CF<sub>2</sub>—CF<sub>2</sub>—) groups. These polymers may vary widely in molecular weight in the form in which they are used for applying to the cutting edge, ranging from a molecular weight of the order of 2000 or even lower to a molecular weight above 2,000,000. The terminal groups at the ends of the carbon chains may also vary, depending, as is well known, upon the method of making the polymer. Polymers made in aqueous media are reported to have terminal carboxyl groups, while others may have hydrogen and/or chlorine atoms attached to the terminal carbon atoms of the chain.

In the case of high molecular weight fluorocarbons, the material may be applied to the blade cutting edge by placing the edge in close proximity to a supply of the fluorocarbon while the latter is heated, to deposit a fluorocarbon coating on the cutting edge. Electrophoresis may also be employed to deposit the material from charged liquid dispersions thereof, or the cutting edge may be sprayed with or simply dipped in the dispersion and allowed to dry. Solid fluorocarbons having a molecular weight in the lower part of the above range may also be applied to the cutting edge by dipping the edge in a dispersion of the particulate fluorocarbon in a volatile liquid medium or by spraying or brushing such a dispersion onto the edge, then evaporating the liquid medium. Among the volatile liquid media which may be used are water, and such Freons as dichlorodifluoromethane, dichlorotetrafluoroethane, trichlorotrifluoroethane, and mixtures thereof.

No matter how the solid fluorocarbon is deposited on the cutting edge, it is essential that the blade carrying the deposited solid fluorocarbon be baked at an elevated temperature of the order of 200° to 750° F. for a period of time sufficient for the fluorocarbon to become firmly adhered to the substrate. The time may vary from less than two minutes up to 48 hours or more depending on the particular fluorocarbon employed, the nature of the substrate, the rapidity with which the coated blade is brought up to temperature, and the temperature achieved. In the case of steel blades, of course, as pointed out above, the blade cannot be heated to temperatures higher than about 400° F. for more than five minutes without some tempering or softening of the blade. In some cases, however, particularly with stainless steel blades, some softening or tempering of the blades can be tolerated since its disadvantages are more than offset by the improvement in shaving effectiveness brought about by the present invention. In general, steel blades when heated to 300° to 320° F. must be baked for at least thirty minutes to achieve optimum results, although longer heating does no harm to the coating. In some cases it is possible to heat the blade before or during the deposi-

tion of the solid fluorocarbon, thus carrying out the baking step simultaneously with the deposition step.

Although the integument on the cutting edge of the blade when the blade is ready for use may be extremely thin, as pointed out above, it is desirable, in order to produce such an integument, that the coating be substantially thicker at the time the baking step begins. Any excess material remaining on the cutting edge which does not bond to the substrate during the baking step is in the form of a loose film which can be readily removed by brushing or rubbing. It is not essential that this excess material be removed before the blade is used.

While the manner of formation of the integument may not be fully understood and applicant does not wish to be bound by the following explanation, it is believed that coalescence of at least some of the solid fluorocarbon particles occurs and that some interaction between the fluorocarbon and the underlying surface such as steel occurs to form a strong bond between the fluorocarbon and the substrate. The resultant thin adherent coating, which is given mechanical support throughout its extent by the underlying blade, reduces the pull during the shaving operation and increases the ease and smoothness of shaving.

The following specific examples are illustrative of the nature of the present invention. Each of the treated blades was found by actual shave tests to have remarkably improved shaving characteristics as compared with a like blade untreated.

#### Example 1

Five hundred milligrams of solid tetrafluoroethylene polymer (pieces cut from Teflon commercial sheet) were placed into a stainless steel lined (stainless steel thickness=0.03 inch) ceramic tube (2" long,  $\frac{7}{16}$ " in diameter, wall thickness  $\frac{1}{16}$ "). The ceramic tube was heated by passing an electric current through a helical tungsten coil made of 40 mil wire with 30 turns in 2 inches of length wound tightly about the outside of the ceramic tube. A Gillette razor blade, previously thoroughly cleaned by washing with trichloroethylene and then dried, was placed with its cutting edge facing the open end of the tube at a distance of four centimeters. This combination was placed in a vacuum chamber evacuated to a pressure of  $10^{-4}$  mm. of mercury. The tungsten coil was heated electrically until the crucible temperature reached 700°-750° F. The current was then controlled so that a pressure of  $3 \times 10^{-4}$  mm. of mercury was maintained during the heating which was continued for four hours. The blade was removed and showed a deposited layer on its cutting edge which exhibited interference colors in the light microscope. The blade was then placed in an air oven at 320° F. for 40 minutes.

#### Example 2

A hardened stainless steel razor blade purchased on the open market was thoroughly cleaned by washing with trichloroethylene and dried; then its cutting edge was dipped into an aqueous colloidal dispersion containing 25% by weight of finely divided solid tetrafluoroethylene polymer (Du Pont's Teflon Clear Finish). Upon removal from the dispersion, the cutting edge of the blade carried with it a coating of the aqueous dispersion which was then dried for one hour at 120° F. in the atmosphere, after which the deposited coating was baked at 750° F. for 7 minutes.

#### Example 3

A finely divided solid fluorocarbon polymer containing a chain of carbon atoms including a plurality of ( $-\text{CF}_2-\text{CF}_2-$ ) groups and also containing a minor proportion (about 1% by weight) of chlorine atoms and a similar proportion of hydrogen atoms with a melting range of 265°-293° C. (Du Pont's Fluorowax TLT-17 Lot No. 2) was dispersed in a 40:60 mixture by weight

of Freon 12 (dichlorodifluoromethane) and Freon 114 (dichlorotetrafluoroethane) to form a dispersion containing 1% by weight of solids. This dispersion was sprayed from a pressure container onto the cutting edge of a Gillette razor blade, cleaned as described in the preceding examples; and the blade was baked at 330° F. in an air oven for 7 hours.

#### Example 4

The fluorocarbon solid described in Example 3 was dispersed in Freon 113 (trichlorotrifluoroethane) to form a dispersion containing 1% by weight of solids. The cutting edge of a Gillette razor blade, cleaned as described above, was dipped into this dispersion and allowed to dry in the atmosphere. The blade was then baked at 320° F. for 16 hours. Similar results were also obtained using similar dispersions containing up to 11% by weight of fluorocarbon polymer.

#### Example 5

The fluorocarbon solid described in Example 3 was deposited onto a Gillette razor blade edge as described in Example 1 except that the temperature of the crucible was maintained at 335° F. and the heating continued for 10 minutes. The blades were removed from the vacuum chamber and showed interference colors on the cutting edge. Similar results can be obtained by heating at a temperature as low as 250° F. for a longer time. The blades were placed in an air oven at 320° F. for 15 minutes. Similar results were also obtained using times up to 16 hours at the same temperature.

#### Example 6

The fluorocarbon solid described in Example 1 was heated in air at atmospheric pressure in a silica crucible to a temperature of 450° C. until a thick white smoke continuously emanated from the crucible. A Gillette razor blade cleaned as described above was held with its edge in the white smoke at a distance of three inches from the crucible for 10 minutes. By reason of its proximity to the crucible, the blade attained a temperature of the order of 300° F. during the deposition of the fluorocarbon on its cutting edge and required no further baking.

Although specific embodiments of the invention have been described herein, it is not intended to limit the invention solely thereto, but to include all of the variations and modifications which suggest themselves to persons skilled in the art.

What is claimed is:

1. A safety razor blade having on its cutting edge an adherent coating comprising a solid fluorocarbon polymer.
2. A safety razor blade having on its cutting edge an adherent coating comprising a solid polymer of tetrafluoroethylene.
3. A safety razor blade as claimed in claim 2 in which said blade is composed of stainless steel.
4. A steel safety razor blade having on its cutting edge an adherent coating comprising a solid polymer of tetrafluoroethylene.
5. A safety razor blade having on its cutting edge an adherent coating comprising a solid polymer containing a chain of carbon atoms including a plurality of ( $-\text{CF}_2\text{CF}_2-$ ) groups.
6. A safety razor blade as claimed in claim 5 in which the molecular weight of said polymer is at least of the order of 2,000.
7. The method of treating a safety razor blade which comprises depositing on its cutting edge a composition comprising a solid fluorocarbon polymer and heating said deposited fluorocarbon polymer to form a coating adherent to said edge.
8. The method of treating a safety razor blade which comprises depositing on its cutting edge a composition comprising a solid polymer of tetrafluoroethylene and

heating said deposited polymer to form a coating adherent to said edge.

9. The method of treating a steel safety razor blade which comprises depositing on its cutting edge a composition comprising a solid polymer containing a chain of carbon atoms including a plurality of ( $-\text{CF}_2-\text{CF}_2-$ ) groups and also including terminal groups selected from the class consisting of carboxyl groups, hydrogen atoms and chlorine atoms, and heating said deposited polymer to form a coating adherent to said edge.

10. The method of treating a steel safety razor blade which comprises depositing on its cutting edge a dispersion in a volatile liquid containing discrete particles of solid polymer containing a chain of carbon atoms including a plurality of ( $-\text{CF}_2-\text{CF}_2-$ ) groups, evaporating said volatile liquid, and heating the resulting deposit at an elevated temperature to form a coating adherent to said edge.

11. The method as defined in claim 10 in which said volatile liquid comprises water.

12. The method as defined in claim 10 in which said heating is carried out for at least 30 minutes at 300° to 330° F.

13. The method as defined in claim 10 in which said volatile liquid is selected from the class consisting of dichlorodifluoromethane, dichlorotetrafluoroethane, trichlorotrifluoroethane, and mixtures thereof.

14. The method of treating a steel safety razor blade

which comprises heating a solid polymer containing a chain of carbon atoms including a plurality of

( $-\text{CF}_2-\text{CF}_2-$ )

groups to a temperature sufficient to vaporize a portion thereof, maintaining a cutting edge of said blade in said vapors to deposit a coating thereon, and heating the resulting deposit to form a coating adherent to said edge.

15. The method as defined in claim 14 in which said heating step is carried out simultaneously with said deposition step.

#### References Cited in the file of this patent

##### UNITED STATES PATENTS

|    |           |                |               |
|----|-----------|----------------|---------------|
| 15 | 2,292,417 | Wetherbee      | Aug. 11, 1942 |
|    | 2,662,065 | Berry          | Dec. 8, 1953  |
|    | 2,707,157 | Stanton et al. | Apr. 26, 1955 |
|    | 2,814,296 | Everett        | Nov. 26, 1957 |
| 20 | 2,855,669 | Duke           | Oct. 14, 1958 |
|    | 2,893,900 | Machlin        | July 7, 1959  |
|    | 2,937,976 | Granahan       | May 24, 1960  |

##### OTHER REFERENCES

25 New Ways to Use Korda "Teflon" Products; Chicago Gasket Co.; Bulletin B-4A; page 1, received in Patent Office June 10, 1952.

UNITED STATES PATENT OFFICE  
CERTIFICATE OF CORRECTION

Patent No. 3,071,856

January 8, 1963

Irwin W. Fischbein

It is hereby certified that error appears in the above numbered patent requiring correction and that the said Letters Patent should read as corrected below.

In the grant, lines 1 to 3, for "Irwin W. Fischbein, of Hyde Park, Massachusetts," read -- Irwin W. Fischbein, of Hyde Park, Massachusetts, assignor to The Gillette Company, of Boston Massachusetts, a corporation of Delaware,--; line 12, for "Irwin W. Fischbein, his heirs" read -- The Gillette Company, its successors --; in the heading to the printed specification, line 3, for "Irwin W. Fischbein, 18 Joyce Road, Hyde Park, Mass." read -- Irwin W. Fischbein, Hyde Park, Mass., assignor to The Gillette Company, Boston, Mass., a corporation of Delaware --; column 2, line 20, for "af" read -- of --; column 3, lines 61 and 74, for "Du Pont's", each occurrence, read -- duPont's --; column 4, line 2, for "from" read -- form --.

Signed and sealed this 23rd day of July 1963.

(SEAL)

Attest:

ERNEST W. SWIDER

Attesting Officer

DAVID L. LADD

Commissioner of Patents